

## UNITED STATES PATENT OFFICE

HOWARD ADLER, OF CHICAGO HEIGHTS, ILLINOIS, ASSIGNOR TO DIVERSEY MANUFACTURING COMPANY, A CORPORATION OF ILLINOIS

## CLEANING METAL SURFACE

No Drawing.

Application filed March 29, 1926. Serial No. 98,404.

The present invention relates to methods for the cleaning of tinned metal surfaces and to detergents suitable for such use, and will be fully understood from the following description, in which specific examples illustrating my invention will be more fully set forth.

Tin plated sheet metal and containers thereof, particularly when used in the handling of food products such as milk, cream or the like, become covered with fatty deposits, for the removal of which it has hitherto been customary to employ alkaline cleaners, such as sodium carbonate, trisodium phosphate, soap powders, borax and the like. Such containers, for example, milk and cream cans, require frequent and thorough cleaning and it has been found that the action of cleaning agents such as those hitherto used result in a corrosion and "checking" of the tin plating. The life of the tin plating is thus greatly lessened, and frequently replating is required.

In accordance with this invention, the checking and corrosion of the tin plating under the action of the cleaning agent of an alkaline nature are prevented by providing during the cleansing, a chromate compound, the presence of which I have found to inhibit or entirely prevent the checking and corrosion of the plating. It is preferred that the chromate compound be incorporated in or admixed with the alkaline cleaning agent from which the cleaning solution for washing the tin plated metal or container is made. If desired, however, the oxidizing agent may be separately incorporated in the alkaline cleaning solution.

The alkaline cleaning agent employed in carrying out this invention may be one of the ordinary alkaline substances used for that purpose; for example, trisodium phosphate, soda ash, soap powder, borax, caustic alkali, or the like. It is preferred, however, that the caustic alkalis such as sodium hydroxide, be

not employed. The chromate compound may be a water soluble chromate or dichromate, preferably of an alkali metal, as sodium, ammonium or potassium dichromate or chromate.

The proportion of the chromate compound relative to the alkaline substance may be greatly varied; thus, proportions as low as 1% of the alkaline cleansing agents are found to substantially inhibit checking or 50 corrosion of the tin plating. Proportions up to 10% may be employed, or even higher if desired, although in general, a suitable range is from 3 to 5% of the oxidizing agent. In preparing the cleansing solution, from  $\frac{1}{2}$  to 55 8 ounces of the cleaning alkaline substance may be employed per gallon of water, together with the desired proportion of the oxidizing agent. Thus, one-half ounce of trisodium phosphate per gallon of water is 60 found to have an appreciable checking action upon tin plate in ten minutes at a temperature of  $65^{\circ}$  C. The addition of 1% of potassium dichromate (based upon the amount of trisodium phosphate) substantially 65 inhibits checking action with concentrations as high as eight ounces per gallon when the application is continued up to sixty minutes at  $65^{\circ}$  C. From 3 to 5% of potassium dichromate completely prevents checking on 70 a treatment of tin plated surfaces with concentrations up to eight ounces per gallon for ten minutes at  $65^{\circ}$  C., and substantially inhibits checking action with concentrations of trisodium phosphate up to eight ounces per 75 gallon when treatment is continued for sixty minutes at  $75^{\circ}$  C.

Soda ash, in concentrations as low as one-half ounce per gallon, causes checking within ten minutes at a temperature at  $65^{\circ}$  C. With 85 this same cleansing agent in concentrations as high as eight ounces per gallon, 1% of potassium dichromate appreciably inhibits checking. Three to five per cent of potassium dichromate substantially prevents checking by 90

soda ash even in concentrations up to eight ounces per gallon and at temperatures of 75° C. when treatment is continued as long as sixty minutes.

5 Other chromates and dichromates, for example, sodium dichromate are similar in their action to potassium dichromate as set forth above.

10 My preferred composition is one containing trisodium phosphate and a chromate compound; for example, 3 to 5% of potassium dichromate or sodium dichromate.

I claim:

15 1. The method of cleaning tinned metal surfaces and inhibiting corrosion of the tin thereof which comprises subjecting such surfaces to the action of a water soluble chromate compound and of an alkaline detergent.

20 2. The method of cleaning tinned metal surfaces and inhibiting corrosion of the tin thereof which comprises subjecting such surfaces to the action of a solution of trisodium phosphate in the presence of a dichromate of an alkali metal.

25 3. The method of cleaning tinned metal surfaces and inhibiting corrosion of the tin thereof which comprises subjecting such surfaces to the action of a solution of trisodium phosphate in the presence of sodium dichromate.

30 4. A detergent for tinned metal surfaces comprising a major portion of a soluble non-caustic alkaline detergent and a minor portion of a water soluble chromate compound.

35 5. A detergent for tinned metal surfaces comprising a major portion of a soluble non-caustic alkaline detergent and a minor portion of a dichromate of an alkali metal.

40 6. A detergent composition for tinned metal surfaces comprising a major portion of trisodium phosphate and a minor portion of sodium dichromate.

45 7. The method of cleaning tinned metal surfaces and inhibiting corrosion of the tin thereof which comprises subjecting such surfaces to the action of a solution of trisodium phosphate in the presence of a dichromate of an alkali metal, the dichromate being present in an amount equal to from one to five percent of the trisodium phosphate.

50 8. The method of cleaning tinned metal surfaces and inhibiting corrosion of the tin thereof which comprises subjecting such surfaces to the action of a solution of trisodium phosphate in the presence of sodium dichromate, the sodium dichromate being present in an amount equal to from one to five percent of the trisodium phosphate.

55 9. A detergent for tinned metal surfaces comprising a soluble non-caustic alkaline detergent and a dichromate of an alkali metal, the alkali dichromate being present in an amount equal to from one to five percent of the alkaline detergent.

60 10. A detergent composition for tinned

metal surfaces comprising trisodium phosphate and sodium dichromate, the sodium dichromate being present in an amount equal to from one to five percent of the trisodium phosphate.

70 11. The method of cleaning tinned metal surfaces which comprises subjecting such surfaces to the washing action of a solution comprising an alkaline detergent in the presence of a chromate compound soluble therein and adapted to protect the tinned surface 75 against corrosion and checking.

HOWARD ADLER.

80

85

90

95

100

105

110

115

120

125

130